

[54] VARIABLE THICKNESS FABRIC MAT FOR RAILWAY TRACK STRUCTURE AND METHOD

[75] Inventor: **Ronald P. Marsh**, St. Louis, Mo.

[73] Assignee: **True Temper Corporation**, Cleveland, Ohio

[21] Appl. No.: 134,787

[22] Filed: Mar. 28, 1980

[51] Int. Cl. 3 B32B 5/06; B32B 5/26; E01B 3/44

[52] U.S. Cl. 238/1; 14/73; 238/2; 405/131; 405/258; 428/77; 428/172; 428/190; 428/212; 428/215; 428/220; 428/284; 428/287; 428/290; 428/311.5; 428/316.6

[58] Field of Search 14/73; 238/1, 2; 104/1 R; 405/131, 258; 428/77, 172, 190, 212, 215, 220, 284, 287, 290, 317

[56] References Cited

U.S. PATENT DOCUMENTS

|           |        |       |        |
|-----------|--------|-------|--------|
| 2,827,412 | 3/1958 | McKay | 428/77 |
| 3,402,227 | 9/1968 | Knee  | 264/64 |
| 3,587,964 | 6/1971 | Cork  | 238/1  |
| 3,598,680 | 8/1971 | Lee   | 19/302 |

|           |         |         |         |
|-----------|---------|---------|---------|
| 3,670,506 | 6/1972  | Goudard | 405/258 |
| 3,765,996 | 10/1973 | Munyon  | 428/172 |
| 4,076,876 | 2/1978  | Bowles  | 428/190 |
| 4,265,398 | 5/1981  | Luebke  | 428/77  |

Primary Examiner—James C. Cannon

Attorney, Agent, or Firm—Baldwin, Egan, Walling & Fetzer

[57] ABSTRACT

A variable thickness fabric mat for use with railroad track right of way beneath the track structure. The mat has a central portion of predetermined thickness, and lateral shoulder portions of a reduced thickness as compared to said central portion, with the central portion being of a predetermined width of adequate dimension to generally completely underlie the railroad track structure. The mat provides a method for transmission of force from a train on the railroad track structure to be spread over a greater area of the underlying earth bearing surface, and with the mat possessing the capability of passing water, and aiding in draining water from the soil beneath the mat, as well as from the top and sides of the track support.

28 Claims, 6 Drawing Figures







Fig 4



Fig 5



Fig 6

## VARIABLE THICKNESS FABRIC MAT FOR RAILWAY TRACK STRUCTURE AND METHOD

This invention relates to general to a resilient mat adapted to underlie a railroad track structure along its right of way, for more uniformly distributing the loads from trains passing thereover to the underlying earth bearing area, and more particularly relates to a variable thickness, fabric mat adapted for underlying the railroad track structure along the right of way and wherein the thicker central portion thereof underlies the track structure, and thinner lateral shoulder portions of the mat extend laterally from such thicker portion. The mat in addition to more uniformly distributing the forces of a train moving on the track structure, to the underlying bearing soil areas, aids in drainage of water from the soil and from above the track support, and helps to stabilize poor support areas of soil. A method of utilizing the mat is also disclosed.

### BACKGROUND OF THE INVENTION

Non-woven mats for use under roads and under railroad track structure along the right of way, are well known in the art. One such arrangement is disclosed in U.S. Pat. No. 3,670,506, dated June 20, 1972 and entitled "Process for Stabilizing Soils", and is directed to a method of utilizing non-woven fabric in poor support areas. Other prior publications include, for instance, an article entitled "Testing of Subgrade Stabilization Fabrics Moves Ahead" in the October 1976 publication of *Railway Track and Structures*. However, to applicant's knowledge, these prior art mats as used in the environments indicated are of generally uniform thickness throughout. Moreover, such prior art mats are generally one unitary member formed of a predetermined substantially uniform thickness of fabric material, and cut into predetermined lengths for use at the site.

Also in a pending U.S. patent application of Robert Luebke, Ser. No. 092,709, filed Nov. 9, 1979, now U.S. Pat. No. 4,265,398, there is disclosed a variable thickness fabric mat for use under railroad track crossings, switches and the like, which patent application is assigned to the assignee of the present application. Various prior publications including aforementioned U.S. Pat. No. 3,670,506 are identified in said Luebke application, and reference by incorporation is made thereto.

The present invention provides a novel variable thickness mat, adapted for use along a railroad track right of way beneath the track structure, so as to more uniformly distribute the force loads from a train to the underlying bearing support soil, and which will not impede drainage. The mat comprises a thicker central portion which underlies the track structure proper, thereby locating the thicker portion where it is most beneficial to the applied loads, and lateral shoulder portions of reduced thickness, as compared to the central portion, with such lateral shoulder portions projecting laterally beyond the confines of the track structure, and adapted to be covered by the ballast bed supporting the track structure.

Accordingly, an object of the invention is to provide a novel variable thickness mat for use along a railroad right of way beneath the track structure for more uniformly distributing the force loads applied to the track structure due to traffic thereover, to the underlying soil bearing areas, and which will not impede drainage, but instead will actually facilitate the latter.

Another object of the invention is to provide a mat of the aforementioned type which is formed of non-woven fabric.

A still further object of the invention is to provide a mat of the above described type which is comprised of a plurality of layers of fabric material, with means connecting the layers together, to form an integral mat member.

A still further object of the invention is to provide a mat of the aforementioned type which includes layers of non-woven fabric combined with at least one layer of woven fabric, together with means connecting the layers together into an integral mat member.

A further object of the invention is to provide a railroad track structure utilizing a mat of the aforesaid type.

A still further object of the invention is to provide a method in a railroad track environment of reducing the stresses thereto utilizing a fabric mat underlying the railroad track structure.

Other objects and advantages of the invention will be apparent from the following description, taken in conjunction with the accompanying drawings wherein:

### BRIEF DESCRIPTION OF THE DRAWINGS

FIG. 1 is a generally perspective, transversely sectioned view of a railroad track structure utilizing the variable thickness mat of the present invention.

FIG. 2 is a generally diagrammatic, broken, elevational view illustrating the variable thickness mat utilized in the railroad track structure of FIG. 1.

FIG. 3 is a generally diagrammatic broken, elevational view illustrating another embodiment of mat.

FIG. 4 is a view generally similar to FIG. 3, but illustrating a still further embodiment of mat.

FIG. 5 is a view generally similar to FIGS. 3 and 4, but illustrating a still further embodiment of mat.

FIG. 6 is a perspective, reduced size illustration of a roll of the mat material, for convenient use on site installation.

### DESCRIPTION OF PREFERRED EMBODIMENTS

Referring now again to the drawings, there is illustrated in FIG. 1 a railroad right of way including track structure 10 comprising ties 12 supported on and embedded in ballast bed 14, with the ties, in the embodiment illustrated, supporting thereon conventional tie plates 16, on which are supported spaced rails 18. Any suitable means can be provided for anchoring or securing the rails and/or tie plates to the ties.

Normally, the ballast bed rests directly on a bearing ground surface 20 which has preferably been previously leveled, as by a bulldozer, track bed plow, undercutter, or the like, and which may or may not provide a good bearing surface. Many times tracks are laid through soft or wet soils which do not provide a good support for the track structure, and therefore, the forces applied to the track structure by the trains moving thereover can affect the track stability, cause undue wear and problems, fouled ballast, and including failure, in the track structure.

Accordingly, in order to attempt to stabilize the ground bearing surfaces and to more uniformly apply the force from the vehicles moving over the track structure, to the underlying soil bearing areas, it is known in the railroad field to use fabric mats including non-woven fabric mats beneath a layer of ballast so as to

more evenly distribute the force loads to the bearing areas.

In accordance with this invention, the mat 22 underlying the track structure 100, comprises a thicker central or track portion 24 and thinner lateral shoulder portions 26 on both sides of the central portion. In the embodiment illustrated in FIG. 2 the mat 22 is formed of a plurality of layers of non-woven synthetic fabric material with the central portion 24 being partially formed of one layer 24a of fabric and the remainder of 10 the central portion and the lateral shoulder portions 26 being formed of a further layer 26a of fabric, which layer 26a extends laterally of both sides of the top layer 24a. In this connection for purposes of underlying conventional United States gauge railroad track structure, the top layer 24a of the central portion may be approximately 90" to 110" in width, while the bottom layer 26a which includes the lateral shoulder portions, may be approximately 150" to 186" in width, with each of the lateral shoulder portions being in the range of from 20 approximately two and one-half feet wide to a little over three feet in width. Means 28 (FIG. 2) is provided connecting or bonding the layers forming the mat 22, together. Such means comprises, in the embodiment illustrated, intertwined fibers of the various layers of 25 fabric, which intertwined fibers are produced by needle punching of the layers, resulting in an integral mat member.

These mechanically interlocked fibers 28 due to the needle punching, may be produced in the conventional manner on needle looms, with the layers of fabric making up the mat being passed into the loom, and being connected as the needle barbs pass downwardly through the layers, interlocking engaged fibers of the mat into individual groups. The end results is a flexible 35 layered, liquid pervious mat of high stability, with the layers thereof secured together by the punched fiber groups as diagrammatically illustrated in FIG. 2 at 28.

Chemical binders of suitable known type may also be utilized between the layers of the mat, for aiding in 40 connecting the layers together. For most purposes, however, and for the purposes of underlying railroad track structure with which the present product is particularly applicable, needle connecting or bonding is adequate, and is preferred, and chemical binders for attaching the mat layers 24a, 26a together are not necessary or even desirable, since such chemical binders may adversely effect the permeability of the mat.

Non-woven fabrics for use in the construction and railroad industries are well known, with such fabrics as aforementioned being utilized in the construction industry for the laying of the automotive roadways as well as in railroad track routes. These known fabrics which are made from a plurality of materials, such as for instance from polyesters, are available from a plurality of companies, including the assignee of the instant invention.

The mats are expeditiously utilizable with poor load bearing soils and form an effective resilient support bed for the railroad track structure in such an environment, to help support and spread the forces from wheeled traffic over the track structure, to the underlying ground bearing area. The mats readily pass runoff water and facilitate the drainage of the water from the railway right of way without impeding drainage. Such drainage is facilitated by the mat 22 from the top of the ballast bed 14 down through the bed, as well as laterally or horizontally through the mat. The lateral shoulder portions 26 of the mat 22 underlying the shoulders 14a of

the ballast bed aid in anchoring the bed in place as well as facilitating drainage of ground water laterally through the mat and from the overlying ballast bed. The mats also actually facilitate by surface tension, the passage of ground water from the underlying bearing ground surface 20, and filter out fine soil particles that might otherwise contaminate the track ballast, thus aiding in maintaining good drainage in the ballast bed, and improved stability of the bearing ground surface.

In the mat structure illustrated in FIGS. 1 and 2, the central track portion 24 is preferably of from about 125 mil to 200 mil thickness, and the lateral shoulder portions are preferably of about 60 to 100 mil thickness. As shown in FIG. 1, the ballast bed 14 preferably fully covers the lateral shoulder portions 26 of the mat.

Layer 24a of the mat is preferably saturated by any suitable means, such as by dipping or spraying, with a synthetic resin-like binder, such as for instance a thermosetting self cross linking acrylic co-polymer emulsion (e.g. Nacryl No. 977 obtainable from Derby Chemical Company of Ashland, Mass.) Thereafter the layer 24a of needle punched non-woven material and binder is subjected to a blast of air operable to drive off the excess binder, and then is oven dried at suitable temperature, to set the resin-like material dispersed throughout the fibers of layer 24a. Such a resin-like impregnating treatment of the non-woven fabric layer 24a does not materially affect the permeability of the fabric to fluid flow, but does substantially increase the tensile strength of the fabric of the mat, as well as increasing the abrasion resistance of the layer 24a.

Thereafter layer 24a is passed through the loom together with aforementioned layer 26a, and is needle punched by the needle barbs of the loom, to mechanically bond or connect layers 24a, 26a together into an integral mat. While layer 26a of the mat could also be impregnated with a resin-like binder material, the latter is not required, and the economics of the situation generally dictates that such not be done.

The finished mat may be provided in any desired lengths. For ease of handling and storage and ease of applying the mat to the railway track, lengths of approximately 300 feet have been found to be convenient and can be rolled, and dropped off at the site of use (FIG. 6) for expeditious handling in laying on the bearing ground surface that has been prepared, such as for instance by leveling, prior to the placing of a layer or bed 14 of ballast thereover. Also such mats can be inserted under existing track structure by the use of the aforementioned undercutter and track bed plow devices, by undercutting an existing track bed and track and inserting the fabric material under the track structure, while the latter is in raised condition, and then redepositing the ballast bed thereon and then lowering the track structure. Such undercutting and ballast redepositing procedures are known in the railway track art.

The choice of the denier per filament or fiber used in the non-woven fabric is governed primarily by the requirements of the end product. However, a denier in the range of 3-9 is preferred for use in the FIG. 2 mat of the invention. In the embodiment of mat illustrated, the fibers from which the mat is formed are of non-continuous or cut type, preferably possessing a length of approximately 3-4 inches. However continuous fibers could also be utilized in formation of the fabric from which the mats are formed. In any event, in the mat of FIG. 2, layer 24a thereof defining in part center portion 24, preferably possesses a weight of approximately 8 to

12 oz. per square yard (this includes the weight of the resin-like binder), while layer 26a which defines shoulder portions 26 preferably possesses a weight of approximately 4 to 6 oz. per square yard.

The following is a table which lists various typical physical characteristics of a polyester fabric mat of the FIG. 2 type embodiment.

| PROPERTY                                                | VALUE                                                                                         | TEST METHOD                            |
|---------------------------------------------------------|-----------------------------------------------------------------------------------------------|----------------------------------------|
| Composition                                             | 100% of Polyester Fiber                                                                       |                                        |
| Construction                                            | Needle Punch Bonding, Variable Thickness Fabric (Binder Impregnation of Track Section of Mat) |                                        |
|                                                         | Shoulder                                                                                      | Track                                  |
| Grab Tensile, lbs                                       | 80                                                                                            | 175                                    |
| Grab Elongation, %                                      | 125                                                                                           | 100                                    |
| @ 10 lbs, %                                             | 40                                                                                            | 5                                      |
| @ 25 lbs, %                                             | 70                                                                                            | 20                                     |
| Trapezoid Tear, lbs                                     | 50                                                                                            | 100                                    |
| Mullen Burst, lbs                                       | 175                                                                                           | +300                                   |
| Thickness, mils                                         | 100                                                                                           | 125                                    |
| Width, inches                                           | 30-                                                                                           | 90                                     |
| Abrasion Resistance (CS 17 Wheel, %)                    | 50                                                                                            | 75                                     |
| Grab Strength                                           |                                                                                               |                                        |
| Retained - 1000 gm weight, 1000 gm weight, 1000 cycles) |                                                                                               |                                        |
| Puncture Resist. lbs EOSD50 U.S. Std.                   | 50                                                                                            | 140                                    |
| Sieve Sizes                                             | 70 mesh                                                                                       | 140 mesh                               |
| Air Perm. cfm                                           | 250                                                                                           | 150                                    |
|                                                         |                                                                                               | ASTM D-737                             |
|                                                         |                                                                                               | (American Society of Testing Mat'l's.) |
|                                                         |                                                                                               | ASTM D-1682                            |
|                                                         |                                                                                               | ASTM D-2263                            |
|                                                         |                                                                                               | Mullen Test                            |
|                                                         |                                                                                               | ASTM D-1777                            |
|                                                         |                                                                                               | Tabor Test                             |
|                                                         |                                                                                               | ASTM D-1175                            |
|                                                         |                                                                                               | Corps. of E. Test                      |

The non-woven synthetic fabrics used in the mat are preferably resistant to attacks by the components normally found in soils and in ground water, and aid in maintaining the ballast layer 14 free of fluids and well drained, any such fluid readily draining both laterally and vertically through the mat. The various layers of the mats may be formed of a polyester which is a stable, long-lived polymer, and preferably is of such porosity that the mat will hold back particles larger than about 70 microns, while generally permitting smaller water born fines to pass through without clogging or binding the fabric.

Referring now to FIG. 3, there is illustrated another embodiment of pad or mat for use beneath railroad track structure. In this embodiment, a plurality of stacked fabric layers 30, 32, 34, 36 are provided, with the bottommost layer 30 comprising the shouldered portions 26 of the mat. In this embodiment, layers 30, 32 and 36 are formed of non-woven synthetic fabric material such as for instance from the aforementioned polyester, while layer 34 may be a relatively heavy denier monofilament synthetic fabric layer, providing a relatively large void section in the mat, thereby facilitating greater drainage of ground water laterally or horizontally through the mat. The heavy denier could be of the order of 10 to 20 denier for the monofilament fiber.

The various layers 30, 32, 34 and 36 are connected together into an integral mat, such as for instance by means of the aforementioned needle punching, as illustrated diagrammatically at 28, and in a similar manner as in the fabrication and connecting of juxtaposed layers of the mat of FIG. 2.

The layers 32, 34 and 36 of the FIG. 3 mat may be impregnated with a resinous binder in the same manner

as aforescribed in connection with layer 24a of the FIG. 2 mat, which provides considerable abrasion resistance to the impregnated mat material, as well as increased tensile strength. Such resin-like binder material is preferably applied to the respective mat layer subsequent to the needle punching thereof to form the layer, but prior to the needle punching of the various layers to form the integral mat structure.

The mat embodiment of FIG. 3 may be particularly useable where the ground support areas encompass considerable surface water, so that the water can more rapidly flow through the mat with reduced obstruction, and especially through the monofilament layer 34. The porosity of the other layers and denier of the filaments thereof may be generally similar to that aforescribed in connection with the layers of the FIG. 2 mat embodiment.

Referring now to FIG. 4, there is illustrated a further embodiment of mat structure. In this embodiment, the non-woven fabric layers 30', 32', 34' and 36' are of variable denier. For instance, layer 30' could be of between 1 to 3 denier per filament while layer 32' could be of between approximately 3 to 5 denier per filament, thus providing a greater strength to layer 32' as compared to layer 30'. Layer 34' could be of 5 to 10 denier per filament, while layer 36' could likewise be of 5 to 10 denier per filament, all of such layers being formed for instance from polyester filament. Also in this embodiment, the various layers 32', 34' and 36' may be impregnated with a resin-like binder as aforescribed for FIGS. 2 and 3 providing improved tensile strength and abrasion resistance to the central portion of the mat during its use beneath railroad track structure.

Referring to FIG. 5, there is illustrated a further embodiment of mat structure. In this embodiment, layers 30", 32" and 36" may be generally similar to the correspondingly numbered layers (except for the suffix prime) in the FIG. 3 embodiment. However, layer 34" in this embodiment comprises a woven synthetic fabric (as opposed to a non-woven synthetic fabric). Such woven layer may be formed of any suitable synthetic material, including polyester, and provides for strength reinforcement of the mat, and also increases its resistance to puncture. Also in this embodiment, the top surface of the uppermost layer 36" may be coated with an abrasion resistance non-apertured coating 40, such as for instance rubber, or plastic, or any other suitable material. Such a coating is adapted to resist wear and/or puncturing by the overlying ballast bed, and may be applied by spraying or by suitable adhesive means, or any other suitable means to provide a good attachment to the underlying confronting top surface of layer 36" of the mat. While coating 40 will substantially prevent the passage of water vertically down through the mat, it has practically no effect on water passage horizontally through the mat, and/or upwardly into the mat from the underlying ground surface 20.

In all of these various embodiments of mats, it will be seen that they provide a generally resilient support for the railroad track structure, and more uniformly distribute the forces applied to the track structure by vehicles moving thereover, to the underlying ground support surfaces thus aiding in equalizing and reducing the stresses applied to the track structure itself. Moreover, these various mat structures actually increase the elimination of water from the underlying and adjacent ground bearing surfaces and the ballast bed, to thereby aid in stabilizing the ground bearing surfaces, and

thereby further aiding in reducing stresses applied to the track structure by traffic moving thereover.

From the foregoing discussion and accompanying drawings it will be seen that the invention provides a novel variable thickness mat adapted for use beneath a railroad track structure, for distributing the load on the track structure over increased area, and a mat structure which includes a thicker central portion adapted to underlie the railroad track structure per se, and lateral shoulder portions of reduced thickness, which are adapted to project laterally outwardly from the thicker central portion, and to underlie the ballast bed.

The invention also provides a mat of the above type in conjunction with railroad track structure, for alleviating stresses applied to the track structure and for improving the condition of the ground bearing surfaces areas which support the track structure, and particularly being operable to improve poor bearing surfaces which have water problems associated therewith.

The invention also provides a novel method of utilizing the mat and more evenly distributing the load from a railroad track and its associated ballast bed, along the railroad track right of way.

The terms and expressions which have been used are used as terms of description, and not of limitation, and there is no intention in the use of such terms and expressions of excluding any equivalents of any of the features shown, or described, or portions thereof, and it is recognized that various modifications are possible within the scope of the invention claimed.

What is claimed is:

1. A method of providing for spreading of the load due to wheeled traffic on a railroad track structure, comprising the steps of placing a variable thickness, elongated, integral, liquid pervious fabric mat of selected length on the earthen support surface so as to cover a selected length of the latter along the railroad right of way, placing a layer of ballast including sloping shoulder portions on said mat and placing the track structure including the ties and the rails on the ballast layer, extending lengthwise of the underlying mat in general alignment therewith, with said mat being of sufficient width so as to substantially completely underlie the transverse extent of the track structure including the ties and the rails, with the mat comprising a thicker central portion where it directly underlies said track structure and thinner lateral portions projecting laterally outwardly beyond said transverse extent of said track structure, said central portion of said mat being of predetermined width and of selected and substantially uniform thickness throughout its length, each of said lateral portions being of lesser thickness and width as compared to the respective thickness and width of said central portion, but being of substantially the same length as said central portion, said mat comprising a plurality of stacked, generally equal length individual layers of fabric material connected together into an integral member and being porous so as to readily pass liquid therethrough but being of such porosity as to prevent the passage of soil particles greater than a predetermined size therethrough, to thereby aid in preventing contamination of said ballast layer, the shoulder portions of said ballast layer overlying and resting on said lateral portions of said mat, said mat extending lengthwise in general alignment with the lengthwise extension of said track structure and said lateral portions being disposed generally laterally of the vertical

planes defining the side confines of the track structure and beneath said shoulder portions of said ballast layer.

2. A method in accordance with claim 1 wherein said mat comprises a plurality of individual layers of nonwoven fabric material with means mechanically connecting the layers together into an integral mat member.

3. A method in accordance with claim 2 wherein at least part of said thicker portion of said mat is impregnated with a resin-like binder material which increases the tensile strength of the mat.

4. A method in accordance with claim 1 including providing the mat in roll form, and unrolling it to said selected length on the earthen support surface for disposal beneath the layer of ballast and the track structure.

5. A variable thickness, elongated, integral synthetic fabric mat pervious to liquid and which includes nonwoven needle punched fabric material, adapted for use beneath a railroad track structure lengthwise of the latter for spreading the load on the track structure over an increased area, said mat comprising a plurality of stacked, generally equal length individual layers of fabric material connected together into an integral member, and being of selected length and comprising a central portion of predetermined width and of selected and substantially uniform thickness throughout its length and lateral portions on both sides of said central portion, each of said lateral portions being of lesser thickness and width as compared to the respective thickness and width of said central portion but being of substantially the same length, said central portion being adapted to extend lengthwise of the track structure beneath the latter with said lateral portions being adapted to be disposed generally laterally outwardly of the vertical planes defining the side confines of the track structure.

6. A mat in accordance with claim 5 wherein said central portion is within the range of approximately 125 to 200 mil thickness and said lateral portions are each within a range of approximately 60 to 100 mil thickness.

7. A mat in accordance with claim 5 which is formed of non-woven polyester fiber.

8. A mat in accordance with claim 5 wherein said central portion includes an abrasion resistant coating on its upper surface.

9. A mat in accordance with claim 5 wherein at least said central portion of said fabric mat has been saturated with a resin-like binder and then subsequently dried.

10. A mat in accordance with claim 5 wherein said means connecting the layers together comprises interlocked fibers from the various layers produced by simultaneous needle punching of juxtaposed individual layers of the mat.

11. A mat in accordance with claim 5 wherein said central portion is of a heavier weight per square yard as compared to the weight per square yard of said thinner lateral portions.

12. A mat in accordance with claim 5 wherein certain of said layers comprises nonwoven needle punched fabric and another of said layers comprises a monofilament fabric, the means connecting the layers together comprising interlocked fibers from the various layers produced by needle punching of juxtaposed layers.

13. A mat in accordance with claim 5 wherein the top surface of said central portion of said mat comprises a layer of abrasion resistant generally non-pervious material, such as for instance rubber.

14. A mat in accordance with claim 5 wherein the grab tensile strength of the central portion of the mat is approximately 175 pounds and the grab tensile strength of the lateral shoulder portions of the mat is approximately 80 pounds.

15. A mat in accordance with claim 5 wherein the central portion has a Mullen burst strength of approximately 300 plus pounds, and said lateral portions of approximately 175 pounds.

16. A mat in accordance with claim 5 wherein said central portion has a puncture resistance of approximately 140 pounds and said lateral portions have a puncture resistance of approximately 50 pounds.

17. A mat in accordance with claim 5 wherein said central portion has an air permeability of approximately 150 cubic feet per minute and said lateral shoulder portions have an air permeability of approximately 250 cubic feet per minute as measured by ASTM D-737.

18. A mat in accordance with claim 5 wherein the width of said central thicker portion is between approximately 90 to 110 inches with the overall width of said mat being between approximately 150 to 186 inches and with said thinner lateral portions each being between approximately two and one half to a little over three feet in width.

19. A mat in accordance with claim 18 which is approximately 300 feet in length.

20. A mat in accordance with claim 5 wherein at least one of said plurality of layers of fabric material, connected together into an integral member, is of a different type of fabric material and possesses a greater liquid permeability as compared to the other of said layers.

21. A mat in accordance with claim 5, wherein the mat comprises at least three stacked layers and the fibers of one of said layers are between approximately 1 to 3 denier, while the fibers of another of said layers are between approximately 5 to 10 denier, and the fibers of another of said layers are between approximately 3 to 5 denier.

22. A mat in accordance with claim 5 wherein one of said layers comprises synthetic woven fabric and the means connecting the layers together comprises interlocked fibers from the various layers produced by needle punching of the layers when the latter are juxtaposed in said stacked condition.

23. In combination with a railroad track structure, including spaced ties, a non-woven, needle punched, liquid pervious, elongated integral fabric mat disposed beneath said structure and extending along beneath said structure lengthwise thereof for a predetermined dis-

10  
5  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880

UNITED STATES PATENT AND TRADEMARK OFFICE  
CERTIFICATE OF CORRECTION

PATENT NO. : 4,311,273  
DATED : January 19, 1982  
INVENTOR(S) : Ronald P. Marsh

It is certified that error appears in the above-identified patent and that said Letters Patent is hereby corrected as shown below:

Column 3, line 4, "100" should read -- 10 --.

Column 3, line 35, "results" should read -- result --.

Signed and Sealed this

Thirteenth Day of April 1982

(SEAL)

Attest:

GERALD J. MOSSINGHOFF

Attesting Officer

Commissioner of Patents and Trademarks